

## UNITED STATES PATENT OFFICE

2,608,476

## COLOR STABLE GASOLINE COMPOSITION

Barney R. Strickland, Westfield, N. J., assignor to  
Standard Oil Development Company, a corpora-  
tion of Delaware

No Drawing. Application January 26, 1949,  
Serial No. 73,013

1 Claim. (Cl. 44—69)

1

This invention relates to a gasoline composition of good color stability. More particularly the invention concerns a gasoline composition consisting of a virgin or paraffinic base stock containing a halogenated hydrocarbon, a phenylenediamine inhibitor and a small amount of cyclohexylamine, or its derivatives. This composition is substantially color stable when exposed to light by virtue of the color stabilizing effect of the cyclohexylamine.

As indicated, this invention concerns a specific fuel composition which without the use of cyclohexylamine, as herein disclosed, is normally color unstable. The fuel base stocks embraced within the scope of this invention are broadly any paraffinic or virgin stock, any hydrogenated stock, or any stock containing substantially no olefins. Within this class of fuel base stocks fall the alkylate types of fuels produced by the reaction of isoparaffins and olefins so as to provide a fuel having substantially no olefins, and hydrogenated polymer types of gasolines formed by the polymerization of low boiling olefins followed by hydrogenation to form hydrocarbons boiling in the gasoline boiling range. The invention does not have application to any hydrocarbon compositions containing substantial quantities of olefins. Thus the invention does not have application to gasoline stocks produced by cracking procedures or by any other refinery process which causes the gasoline to have an appreciable olefin content unless further processed to eliminate the olefins.

As a further limitation of the composition of this invention, it is necessary that the fuel contain halogen compounds. In its broadest sense the halogen compound can be present in any form although in a practical sense the halogen compound is normally used in a gasoline as a "lead scavenging agent." Suitable lead scavenging agents are, generally speaking, any halogenated hydrocarbons, as this class of compounds has the property of being reactive with lead anti-knock agents in the gasoline to yield volatile lead compounds which can be evacuated from the engine. As the name suggests, lead scavenger agents are employed to decrease lead deposits in an engine and other undesirable effects otherwise resulting from the presence of lead anti-knock agents. As the present time the scavenging agents which are employed commercially are mixtures of ethylene dibromide and ethylene dichloride, although many other scavenging agents can be employed such as brominated C<sub>6</sub>—C<sub>8</sub> aromatics, mono-, di-, and tri-halogenated paraffins, etc. As stated, therefore, the compositions of this invention are fuel compositions containing

2

halogenated compounds, and specifically containing halogenated hydrocarbons used as lead scavenging agents in conjunction with lead anti-knock agents. Again the anti-knock agent to be employed may be any of the lead alkyl compounds normally employed as lead scavenging agents. While tetraethyllead is the anti-knock agent ordinarily employed, if desired the agent may be tetramethyllead, trimethyllethyllead, di-10-methyldiethyllead, methyltriethyllead, triethyl-n-propyl lead or other alkyl lead compounds.

This invention is not limited to compositions containing any particular proportion of halogenated compounds or of lead anti-knock agents. 15 However aviation gasolines generally contain quantities of tetraethyllead up to 4.6 ml. tetraethyllead per gallon together with one theory of ethylene dibromide; one theory being the amount of ethylene dibromide which would completely react with all of the lead present. Automobile gasolines generally contain quantities of tetraethyllead up to 3 ml. per gallon together with one theory ethylene dichloride and 0.5 theory ethylene dibromide.

25 The compositions of this invention also contain a specific class of anti-oxidants; this class of anti-oxidants is the phenylenediamines and particularly the N,N'-dialkyl-p-phenylenediamines. Suitable phenylenediamines which are, 30 or may be, employed are N,N'-di-sec-butyl-p-phenylenediamine and N,N'-di-n-butyl-p-phenylenediamine. Generally gasolines contain up to about four pounds per 5000 gallons of the anti-oxidant.

35 So far as is presently known this invention has no application to compositions containing anti-oxidants other than those selected from the class of phenylenediamines.

The color stabilizing agent of this invention is 40 cyclohexylamine, or derivatives of this compound such as derivatives having an alkyl group or groups on either the carbon atoms or on the nitrogen atom. An example would be N-methyl-cyclohexylamine. Such derivatives having alkyl groups containing one to eight carbon atoms may be used. The quantity of cyclohexylamine or its derivatives to be employed is about 0.05 to 0.2 pound per 5000 gallons of gasoline composition, or about 0.0002 to 0.0006 weight percent.

45 50 As described, therefore, this invention relates to non-olefinic hydrocarbon fuel compositions containing phenylenediamine anti-oxidants and containing halogen atoms normally present in the form of lead scavengers together with lead anti-knock agents. In order to render this composition color stable, a small amount of cyclohexylamine is mixed with the composition. By

this means the indicated composition, which without the presence of cyclohexylamine would be color unstable in the presence of light, is rendered substantially color stable. The invention is, therefore, of particular application to gasolines which are exposed to light during storage, or during marketing. For example, the composition of this invention is particularly adapted for use in gasoline pumps having transparent bowls. As will be disclosed, a composition of the nature indicated not containing cyclohexylamine is normally subject to rapid and marked coloration generally causing the gasoline to have a pink color. Discoloration apparently is due to the action of sunlight on the composition, as heating the gasoline does not cause this discoloration. It is theorized that light causes a photochemical reaction of the halogen present in the composition with the phenylenediamine inhibitor. It is probable that sunlight causes release of halogen atoms from the scavenging agent which then combine with the inhibitor to form the pink coloration, or more precisely to form a pink precipitate which is visually apparent. Upon analysis it has been found that this pink precipitate contains 37.1% bromine content when the gasoline composition contained N,N'-di-sec-butyl-p-phenylenediamine and ethylenedibromide as the scavenging agent. Insofar as the combination of one atom of bromine with one molecule of the inhibitor would result in a bromine content of 26.7%, and the combination of two atoms of bromine would give a bromine content of 42.1%, it appears that the precipitate contains almost two atoms of bromine per molecule of the inhibitor.

In order to fully understand the nature of this invention and to appreciate the scope of the invention, the following data and examples are presented.

In order to determine the source of the pink coloration encountered in compositions of the general nature described, a series of tests were made employing compositions of varying nature. Thus the compositions tested contained base stocks of varying kinds, contained different antioxidants, contained different color dyes, and contained different potential color change inhibitors. Presented in Table I below are a series of tests which establish that the undesirable color instability which may arise is not due to dyes which may be present in the gasoline.

TABLE I

| Sample                                                                                              | Color     |                                   |
|-----------------------------------------------------------------------------------------------------|-----------|-----------------------------------|
|                                                                                                     | Initially | After 3 Hour Exposure To Sunlight |
| (a) Alkylate <sup>1</sup>                                                                           | Clear     | Clear                             |
| (b) Alkylate+4.6 ml. Blue TEL/gal. <sup>2</sup>                                                     | Blue      | Blue                              |
| (c) Alkylate+4.6 ml. Blue TEL/gal.+1# N,N'-di-sec-butyl-p-phenylenediamine/5 M gal.                 | do        | Purple                            |
| (d) Alkylate+1# N,N'-di-sec-butyl-p-phenylenediamine/5 M gal.                                       | Clear     | Clear                             |
| (e) Alkylate+1# N,N'-di-sec-butyl-p-phenylenediamine/5 M gal.+1 drop EtBr <sub>2</sub> Per 100 ccs. | do        | Pink                              |
| (f) Alkylate+1# N,N'-di-sec-butyl-p-phenylenediamine/5 M gal.+4 ml. Q TEL/gal. <sup>3</sup>         | Yellow    | Orange                            |
| (g) Alkylate+4 ml. Q TEL/gal. <sup>3</sup>                                                          | do        | Yellow                            |

70

<sup>1</sup> Similar data obtained with virgin naphtha.<sup>2</sup> Blue Commercial Ethyl fluid containing a blue dye and 1 theory of EtBr<sub>2</sub> based on pure TEL.<sup>3</sup> Q TEL fluid containing a yellow dye and 1 theory of EtCl<sub>2</sub> plus 0.5 theory EtBr<sub>2</sub> based on pure TEL.

The first composition tested, as indicated in

Table I, was an alkylate gasoline base stock having a boiling range of about 100 to 350° F., and having been obtained by reaction between isobutylene and isobutane in the presence of sulfuric acid catalyst at about 60° F. This alkylate was initially clear and water white. After exposing the alkylate to the action of sunlight for three hours, it was found that the color did not change, and that the alkylate remained clear and uncolored.

The composition (b) indicated in Table I consisted of this alkylate plus 4.6 ml. per gallon of a commercial tetraethyllead fluid normally used in aviation gasolines. This tetraethyllead fluid is colored for identification purposes with a blue dye of an unascertained composition and contains one theory of ethylene dibromide as the lead scavenging agent. In other words the tetraethyllead fluid contains an amount of ethylene dibromide sufficient to stoichiometrically react with the lead present. By virtue of the blue dye contained in the tetraethyllead fluid the composition (b) initially had a blue coloration. After exposure to sunlight it was found that the coloration of the gasoline had not changed, and that the color of the gasoline remained the same blue.

Composition (c) of Table I was the alkylate identified plus 4.6 ml. per gallon of the blue tetraethyllead fluid employed in composition (b) plus 1 pound of N,N'-di-sec-butyl-p-phenylenediamine per 500 gallons of composition. Again the initial color of composition (c) was blue due to the blue dye present in the tetraethyllead fluid. However, after exposing the composition to sunlight a color change was observed. The color apparently resulted from pink color bodies in combination with the blue dye to yield an apparent purple color. It is apparent from these examples, that is, the tests of compositions (a), (b), and (c) of Table I, that the blue dye employed in the commercial tetraethyllead fluid used was not responsible for the discoloration of the alkylate on exposure to sunlight. In order to determine if the inhibitor N,N'-di-sec-butyl-p-phenylenediamine was responsible for this effect, the compositions (d), (e), and (f) were then tested.

The composition (d) consisted of the alkylate plus 1 pound of the inhibitor, N,N'-di-sec-butyl-p-phenylenediamine, per 5000 gallons of alkylate. It was found that the initial color of composition (d) was clear and uncolored, and that no color change occurred after exposure to sunlight.

However as shown by the test of composition (e) in Table I, employing the composition (d) to which was added one drop per 100 ccs. of ethylene dibromide, it was found that while the initial color of composition (e) was clear and uncolored, a pink coloration developed after exposure to sunlight.

As a further test, composition (e) was mixed with 4 ml. per gallon of a yellow tetraethyllead fluid to obtain composition (f) indicated in the table. The yellow tetraethyllead employed was again a commercially-prepared lead fluid for use in automotive gasolines and contains an unidentified yellow dye to identify the fluid, together with one theory of ethylene dichloride and 0.5 theory of ethylene dibromide based on the tetraethyllead content of the fluid. It was found that the composition (f) had an initial color which was yellowish due to the dye employed, and it was found that after exposure to sunlight a color change occurred which again

appeared to be due to the presence of pink color bodies which resulted in an over-all color which was more or less orange. Again, therefore, a color change was noted in an alkylate composition containing the inhibitor N,N'-di-sec-butyl-p-phenylenediamine and a halogen compound. In order to entirely eliminate the possibility that this color change was due to change in the color of the dye present in the lead fluid, the composition (g) was prepared.

Composition (g) consisted of the alkylate plus 4 ml. per gallon of the tetraethyllead fluid employed in composition (f). In other words composition (g) corresponded to composition (f) except that the inhibitor N,N'-di-sec-butyl-p-phenylenediamine was not present. It was found that the initial color of composition (g) was yellow and that no color change occurred after exposure to sunlight.

From tests of the nature indicated in Table I it was established that the pink coloration encountered in gasolines exposed to sunlight is not due to the discoloration of dyes present in the gasoline, such as the yellow and blue dyes commercially utilized in tetraethyllead fluids. Further experiments were conducted of the same nature as indicated in Table I utilizing virgin naphtha stocks rather than the alkylate employed in Table I. Again it was found that data were obtained corresponding to those presented for the alkylate compositions.

Insofar as the data of Table I indicates that the inhibitor employed is responsible for the objectionable pink discoloration encountered, a series of tests were conducted in which a variety of inhibitors other than a phenylenediamine

consisted of virgin naphtha base stocks containing tetraethyllead fluid containing a blue dye. The virgin naphtha employed was a low sulfur virgin naphtha having a boiling range of about 200 to 350° F., 4 ml. of the tetraethyllead fluid were employed per gallon, and the fluid utilized was a commercial fluid colored with a blue dye containing an addition to the lead tetraethyl and the blue dye one theory of ethylene dibromide. As indicated by composition (a) of Table II, this composition had an initial blue color which was unaltered upon exposure to sunlight.

The test of composition (b) indicates that when composition (a) was mixed with 1 pound per 5000 gallons of N,N'-di-sec-butyl-p-phenylenediamine, while the inhibitor did not change the initial blue color of the gasoline, discoloration did occur after exposure to sunlight, resulting in a purplish tinge in the gasoline. As represented by compositions (c), (d) and (e) of Table II, this discoloration was not encountered when employing normal-butyl-para-aminophenol, isobutyl-para-aminophenol or 2,6-di-tert-butyl-4-methylphenol.

The data of Table II, therefore, together with that of Table I, substantiates the fact that the pink coloration developed in the compositions tested was due to the combination of non-olefinic naphtha, a phenylenediamine inhibitor, and a halogen compound.

Further experiments were then conducted employing base stocks other than substantially saturated paraffinic stocks. In particular the stock employed was one containing a substantial proportion of cracked gasoline as indicated in Table III.

TABLE III  
Effect of inhibitors on the sunlight stability of gasolines

| Gasoline                                                 | Initial | In Direct Sunlight, Hrs. |                       |                       |
|----------------------------------------------------------|---------|--------------------------|-----------------------|-----------------------|
|                                                          |         | 0.50                     | 1.50                  | 3.50                  |
| Gasoline A+2 ml. TEL <sup>1</sup> —Uninhibited.          | Orange  | Orange                   | Orange                | Orange                |
| +2, 6-di-tert-butyl-4-methylphenol, 2 lbs./5000 gal.     | do      | do                       | do                    | Do.                   |
| +N, N'-di-sec-butyl-p-phenylenediamine, 2 lbs./5000 gal. | do      | do                       | do                    | Do.                   |
| Virgin Naphtha+4 ml. TEL <sup>2</sup> Uninhibited.       | Blue    | Blue                     | Blue, Slightly Cloudy | Blue, Slightly Cloudy |
| +2, 6-di-tert-butyl-4-methyl-phenol, 2 lbs./5000 gal.    | do      | do                       | do                    | Do.                   |
| +N, N'-di-sec-butyl-p-phenylenediamine, 2 lbs./5000 gal. | do      | Pink                     | Pink                  | Pink                  |

<sup>1</sup> Fluid contained ethylene dichloride and ethylene dibromide and orange dye.

<sup>2</sup> Fluid contained ethylene dibromide.

were employed. These tests are indicated in Table II.

TABLE II

| Sample                                                                                       | Color     |                                 |
|----------------------------------------------------------------------------------------------|-----------|---------------------------------|
|                                                                                              | Initially | Exposed to Sunlight for 3 Hours |
| (a) Virgin naphtha+4 ml. Blue TEL <sup>1</sup> gal.                                          | Blue      | Blue                            |
| (b) Virgin naphtha+4 ml. Blue TEL <sup>1</sup> gal. + N, N'-di-sec-butyl-p-phenylenediamine. | do        | Purple                          |
| (c) Virgin naphtha+4 ml. Blue TEL <sup>1</sup> gal. + n-butyl-p-aminophenol.                 | do        | Blue                            |
| (d) Virgin naphtha+4 ml. Blue TEL <sup>1</sup> gal. + isobutyl-p-aminophenol.                | do        | Do.                             |
| (e) Virgin naphtha+4 ml. Blue TEL <sup>1</sup> gal. + 2,6-di-tert-butyl-4-methylphenol.      | do        | Do.                             |

<sup>1</sup> Blue commercial ethyl fluid containing a blue dye and one theory of ethylene dibromide based on pure TEL.

It will be observed that the compositions tested

for comparative purposes, gasoline A containing cracked constituents and being a commercial production motor gasoline was tested together with a virgin naphtha. It was found that gasoline A was initially orange, and remained orange after 3½ hours of exposure to direct sunlight. Furthermore, this gasoline showed no color change after exposure to sunlight when N,N'-di-sec-butyl-p-phenylenediamine and when 2,6-di-tert-butyl-4-methylphenol were added to the gasoline. On the other hand the virgin naphtha gasoline tested was initially blue and developed no color change on exposure to sunlight either when uninhibited or when containing 2,6-di-tert-butyl-4-methylphenol. However, when the virgin naphtha gasoline contained the phenylenediamine inhibitor, a pink coloration did develop in the gasoline when exposed to sunlight for a period of one-half hour, or longer. It is, therefore, apparent from the data of Table III that the pink discoloration developed when employing a

phenylenediamine inhibitor only develops when the gasoline base stock contains substantially no olefins. This is a logical result in view of the probable mechanism of the discoloration as formerly stated. If, as theorized, the coloration is due to the photochemical reaction of halogens with *N,N'*-di-sec-butyl-p-phenylenediamine, it is possible that the presence of olefins would prevent the reaction of halogens with the inhibitor and permit a preferential reaction of the halogens with the olefins. As stated, therefore, the gasoline compositions embraced in this invention are gasoline base stocks containing substantially no olefinic constituents.

As presented, therefore, from the data of Tables I, II and III, it appears that the objectionable pink discoloration which develops upon exposure to sunlight of virgin naphtha or non-olefinic compositions, is due to the discoloration of *N,N'*-di-sec-butyl-p-phenylenediamine on reaction with halogen compounds. In order to determine suitable compounds to inhibit this discoloration, a series of tests were then conducted as reported in Table IV, employing a variety of possible color stabilizers.

TABLE IV

| Alkylate+4 ml. Blue TEL/gal.+1 lb. <i>N,N'</i> -di-sec-butyl-p-phenylenediamine/5#M gal. | Color After<br>1 Hour<br>Sunlight<br>Exposure |
|------------------------------------------------------------------------------------------|-----------------------------------------------|
| a. As is.....                                                                            | Pink.                                         |
| b. +0.1 lb. cyclohexylamine.....                                                         | Blue.                                         |
| c. +0.42 lb. cresylic acids.....                                                         | Purple.                                       |
| d. +0.84 lb. cresylic acids.....                                                         | Do.                                           |
| e. +0.42 lb. n-butyl-p-aminophenol.....                                                  | Do.                                           |
| f. +0.84 lb. n-butyl-p-aminophenol.....                                                  | Do.                                           |
| g. +0.42 lb. lecithin.....                                                               | Do.                                           |
| h. +0.84 lb. lecithin.....                                                               | Blue.                                         |
| i. +0.42 lb. cyclohexylamine.....                                                        | Do.                                           |
| j. +0.84 lb. cyclohexylamine.....                                                        | Do.                                           |
| k. +0.21 lb. cyclohexylamine.....                                                        | Do.                                           |
| l. +0.42 lb. tributylamine.....                                                          | Do.                                           |
| m. +0.42 lb. pyridine.....                                                               | Purple.                                       |
| n. +0.42 lb. phenol.....                                                                 | Do.                                           |
| o. +0.42 lb. alpha-naphthylamine.....                                                    | Do.                                           |
| p. +0.42 lb. naphthenic acids.....                                                       | Do.                                           |
| q. +0.42 lb. aniline.....                                                                | Do.                                           |
| r. +1.2 lb. alpha-naphthol.....                                                          | Do.                                           |
| s. +0.42 lb. t-butyl catechol.....                                                       | Do.                                           |
| t. +0.42 lb. pyrogallol.....                                                             | Do.                                           |

The composition tested was alkylate A of Table I with 4 ml. of tetraethyllead per gallon and one pound per 5000 gallons of *N,N'*-di-sec-butyl-p-phenylenediamine. This composition originally had a blue color due to the presence of blue tetraethyllead fluid dye, but after exposure to sunlight for 1 hour, pink color bodies developed in the gasoline as indicated by marked color change. Reported in tests (b) through (t) of Table IV are the results of combining the compounds indicated with the alkylate containing the tetraethyllead fluid and phenylenediamine. It will be observed that of all the compounds tested none of them, with the exception of cyclohexylamine was successful in stabilizing the color of the gasoline when exposed to sunlight.

Having now fully described this invention, what is claimed is:

A paraffinic base gasoline composition containing 0 to 4.6 milliliters per gallon of tetraethyl lead, about one to one and one-half theories of a halogenated hydrocarbon lead scavenging agent, based on tetraethyllead, a quantity of *N,N'*-di-sec-butyl-p-phenylenediamine greater than 0 and less than about four pounds per 5000 gallons, and about 0.05 to 0.2 pound per 5000 gallons of cyclohexylamine.

BARNEY R. STRICKLAND.

## REFERENCES CITED

The following references are of record in the file of this patent:

## UNITED STATES PATENTS

| 35 | Number    | Name       | Date          |
|----|-----------|------------|---------------|
|    | 2,111,307 | Bartram    | Mar. 15, 1938 |
|    | 2,436,838 | Von Bramer | Mar. 2, 1948  |
|    | 2,498,630 | Thompson   | Feb. 28, 1950 |